

## UNITED STATES PATENT OFFICE

2,652,343

## PHOTOGRAPHIC DYE SOLUTION

Clarence E. Payne, San Francisco, Calif.

No Drawing. Application December 22, 1947,  
Serial No. 793,327

14 Claims. (Cl. 106—287)

1

This invention relates to, and it is an object to provide, improvements in the art of varying the printing qualities (or color) of a gelatin supported photographic image through controlled imbibition of a dye or dyes from a high viscosity solution through the agency of differences of osmotic pressures.

While the invention is described herein mainly in relation to the modification, by dye, of the density of an image of a gelatine type photographic negative in order to improve its printing quality, the invention is otherwise useful for controlled dye application to the emulsion of prints, diapositives, lantern slides, or the like.

It is also an object of the invention to provide novel processes, chemicals, and techniques to offset or nullify the undesirable side effects normally encountered in the application of dyes to photographic gelatin.

Ever since the introduction into photography of gelatino-silver bromide emulsions, photographers have sought some easy method of selectively increasing the densities of portions of their negatives in order to secure better printing balance or to change at will the contrast of areas within a negative.

The most acceptable approach to the problem was to add to the gelatin some stain or color which would hold back a portion of the printing light while permitting the desired amount of effective illumination to reach the printing paper.

For purposes of enlarging, such stain or color should be free of structure, and it should dye the gelatin uniformly and smoothly without mottling or fringing, and without disturbing the normal physical characteristics of the gelatin.

There has been available only one technique which was workable within the limits of commercial practice. This consisted of the use of a water soluble dye made up in extremely dilute solution and applied with a small brush, the brush being wiped almost dry before being applied to the gelatin; the brush then being kept in constant motion in contact with the gelatin until it no longer gave up color. The process was then repeated. This slow and tedious method was continued until the desired depth of tone was reached. Only an experienced worker, continuing the process over a considerable period of time, could achieve anything approaching a uniform stain over a large area.

The reason for this painstaking process is that gelatin immediately takes up an aqueous dye solution and, if a solution containing more than a trace of dye is used, with the above outlined

technique, uniform tones are impossible to achieve.

It is thus an additional object of the invention to provide a liquid vehicle which will act as a satisfactory carrier for the dye, and as a restrainer of the rate of imbibition, while incorporating chemicals to control any undesirable side effects.

To this end investigation was made into the oxy-organic compounds of the nature of aliphatic dihydroxy alcohols (i. e. glycols), e. g. diethylene glycol, etc.

A simple aqueous dye-glycol solution was unsatisfactory for several reasons. The surface tension was too high for easy applications; the solution retracted and would not hold a line; the imbibition rate was erratic; the gelatin formed a permanent distortion ring at the gelatin-solution atmosphere juncture; some of the glycol appeared to enter the gelatin and required a prolonged period to evaporate; and the treated film distorted under the heat of the printing light, producing serious Newton's rings in glass sandwich negative carriers.

Chemical additions were then provided which eliminated these undesirable effects.

The dye solution of this invention is red for best density regulation, is quickly applied, readily controlled, and instantly removed when the desired depth of color is obtained. The treated gelatin is smooth, tough, and relatively scuff-proof, and—when treated with the dehydrator-cleaner-hardener which is part of the process and technique—is immediately ready for printing. The gelatin is harder, lies flater, and shows less tendency to produce Newton's rings in a glass negative carrier than before treatment. The time required to secure a moderate stain, stopping about 50% of the printing light, is no more than two minutes.

Another object of the invention is to provide a solution and process which leaves no chemical nor reaction by-product in the gelatin, which might in time deteriorate either the gelatin or the silver image.

It is a peculiar and important characteristic of the present dye solution that there is an interval following application to the gelatin during which little or no dye is transferred, and it is possible to so adjust the solution that the operator will have ample time in which to spread the solution over a considerable area and to work in the details of an irregular contour without sacrificing any uniformity in the dye deposit.

A further object of the invention is to produce

a practical and reliable photographic dye solution and process, which are exceedingly effective for the purpose for which they are designed.

These objects are accomplished in the manner as will fully appear by a perusal of the following specification and claims.

Referring now to the details of the invention, the dye formula comprises initially separate solutions, as follows:

*Solution A*

|                                                                            | Cc.  |
|----------------------------------------------------------------------------|------|
| Dilute C. P. acetic acid, sp. gr. 1.040                                    | 33.5 |
| Acetaldehyde (Acetaldehyde boils at 69° F.)                                |      |
| Therefore, ingredients and utensils for this solution must be below 60° F. | 16   |
| Diethylene glycol                                                          | 2000 |
| Make up 24 hours before use.                                               |      |

*Solution B*

|                                                                                                          |           |
|----------------------------------------------------------------------------------------------------------|-----------|
| Brilliant Scarlet 3R (C. I. 185, page 42) (National Aniline Division, Allied Chemical & Dye Corporation) | grams 100 |
| Distilled water (boiling)                                                                                | cc 900    |
| When cool, qs                                                                                            | cc 1000   |
| A saturated solution, decant if necessary.                                                               |           |

*Solution C*

|                                                                                                                  |          |
|------------------------------------------------------------------------------------------------------------------|----------|
| Food, Drug, and Cosmetic Green No. 3 (Fast Green) (National Aniline Division, Allied Chemical & Dye Corporation) | grams 15 |
| Distilled water (boiling)                                                                                        | cc 980   |
| When cool, qs                                                                                                    | cc 1000  |

*Solution D*

|                                                                                                    |          |
|----------------------------------------------------------------------------------------------------|----------|
| Food, Drug, and Cosmetic Blue No. 1 (National Aniline Division, Allied Chemical & Dye Corporation) | grams 15 |
| Distilled water (boiling)                                                                          | cc 980   |
| When cool, qs                                                                                      | cc 1000  |

*Solution E*

|                                     | Cc. |
|-------------------------------------|-----|
| Distilled water                     | 980 |
| Aerosol OT, commercial 10% solution | 20  |

Make up several hours before use.

The above described separate solutions are combined in the following amounts, with stirring, to produce the complete dye solution:

|            | Cc. |
|------------|-----|
| Solution A | 180 |
| Solution B | 60  |
| Solution C | 17  |
| Solution D | 12  |
| Solution E | 100 |

Bottle tightly and agitate occasionally for twenty-four hours, and thereafter add:

Solution A 80 cc.

with stirring. Bottle and agitate occasionally for twenty-four hours. Some improvement in working qualities appears with further aging.

The process also contemplates the use of a dehydrating-cleaning-hardening solution of the following formula:

|                          | Cc. |
|--------------------------|-----|
| Isopropyl alcohol (pure) | 500 |
| Amyl acetate, purified   | 4   |
| Acetaldehyde             | 10  |
| Distilled water          | 20  |

Ingredients and utensils below 60° F.

The dehydrating-cleaning-hardening solution, and the complete dye solution, are used in the process as now described.

The cleaning solution is applied to the gelatin surface of a negative, or the like, with a pledge.

of cotton, the surface is mopped for thirty seconds or more, and then the solution is removed by buffing with a dry puff of cotton.

Thereafter the dye solution is flowed upon the surface of the gelatin with a soft brush of a size suited to the area to be covered. The dye solution is pooled and puddled over the area being dyed and it is left on the gelatin for a number of minutes predetermined by test upon the particular material in use; such number of minutes giving a density of dye which will produce the desired effect upon the image being treated. At the end of the predetermined interval the dye solution is squeegeed from the gelatin with a roll of cotton, no great care being necessary to avoid damaging the gelatin surface.

Then, the cleaning solution is again applied, in somewhat greater quantity, and after a minute or more, is buffed off. This buffing technique is important, as tests indicate that the hardening and conditioning of the gelatin take place at the evaporating point. The cleaning solution has a pronounced dehydrating effect and where deep stains are placed in the gelatin, with increased moisture absorption, a second application of the dehydrator-cleaner-hardener is indicated, whereupon the negative, or the like, is ready for use.

The dye formula is critical in the following respects:

*The carrier.*—Diethylene glycol is absorbed by gelatin very slowly, and its absorption rate is increased as the water content of the solution is increased. It is a critical factor that the water content must be held low in relation to the diethylene glycol, and some means other than increased water be used to speed imbibition. This latter effect is achieved through the wetting agent, Aerosol OT.

Viscosity-surface tension is controlled by the relationship; diethylene glycol-water-Aerosol OT. The viscosity must be sufficient to prevent spreading. The surface tension must be at a minimum so that the solution will lie flat and not retract as the gelatin takes up the water and changes the diethylene glycol-H<sub>2</sub>O balance.

The viscosity is supplied by the diethylene glycol and the interaction of the other ingredients. The surface tension is reduced and controlled by the commercial wetting agent, Aerosol OT (sodium di-octyl sulfosuccinate). It should be noted here that some control can be exercised over the imbibition rate by varying the diethylene glycol-Aerosol OT solution balance, but the variation must not be sufficient to destroy the good working qualities of the formula.

*Acidity.*—The pH of the solution is controlled by the acetic acid. The pH must be held within narrow limits close to the iso-electric point of gelatin (4.7). The pH of the complete dye solution is 4.43. This acidity eliminates edge distortion, prevents undue swelling of the gelatin and promotes uniform imbibition of the dyes. The acetic acid exerts an unexplained control over the buckling tendency of the film under heat. Excess acid causes creeping of dye. Insufficient acid does not control side effects.

*Hardening and restraining agents.*—None of the gelatin hardening agents used in the customary practices of photography are suitable for the purposes of this formula. As with the other ingredients (except the dyes), the hardening agent must be volatile, yet must be of sufficient stability for the practical purposes of storage and use. Acetaldehyde polymers (aldol condensation), such as paraldehyde or aldol, have been

found by me to meet these requirements and are readily formed from the parent chemical in the solution. In the present embodiment it can be anticipated that an acetaldehyde-paraldehyde equilibrium will be set up, a buffering effect being secured which, when disturbed, will release the highly volatile acetaldehyde from the more stable polymer. In addition to acting as a hardening agent, the acetaldehyde serves to reduce, and so control, the imbibition rate. This latter effect is pronounced. An excess of acetaldehyde stops the action altogether. It is therefore a critical factor that the minimum amount of acetaldehyde which produces a satisfactory hardening is not great enough to unduly inhibit the imbibition rate. It has been found that certain esters have a pronounced hardening effect upon gelatin, and this is true even though the ester has but a very limited solubility in water. Two of these are made use of in this process: amyl acetate and sodium di-octyl sulfosuccinate (aerosol OT). It is worth noting that a solution containing diethylene glycol, acetic acid and acetaldehyde, adjusted with water to the same dilution as is the final formula, does not temper the gelatin so satisfactorily as the complete solution containing the ester, Aerosol OT).

*Nature of the dyes.*—Suitable dyes are water soluble acid dyes, substantive to gelatin, which are compatible with the other substances in solution and which, when mixed for special spectral characteristics, must have identical capillarities under the conditions of use.

All of the chemicals outlined above combine to form a homogeneous, stable solution which, through osmotic pressure, transfers dye at a uniform, controlled rate into photographic gelatin, whether that gelatin be the silver emulsion of a negative, or the anti-halo, non-curling gelatin backing of a negative, or the emulsion of a print or of a diapositive or lantern slide, whether of silver image or of its colored chemical reaction products, or of images in gelatin formed wholly or partly of dye or dyes.

It is apparent, therefore, that the process may be used to modify the colors of a colored film or a diapositive, or a colored print which carries the coloring materials in a gelatin medium, and that for such purpose the dye or dyes can be modified or substituted to meet specific requirements.

The dehydrating-cleaning-hardening solution serves a multiple purpose. Used prior to the application of the dye solution, it cleans the surface of the gelatin, removing grease and foreign material which might interfere with the action of the dye. It brings about a change in the surface of the gelatin by producing a glass-like hardness which resists scuffing even when the gelatin has absorbed considerable water. It introduces a minute quantity of amyl acetate, a hydrophobic agent, which serves an important role in controlling the behavior of the dye solution at the gelatin-atmosphere juncture. This solution, used after the application of the dye solution, rapidly dehydrates the gelatin, further conditioning, and hardening it so that within a minute or two following its application the negative, diapositive, or print is ready for use. It serves further, when multiple applications of dye are to be made, to act as a controlling and inhibiting agent, so that dyed areas which may contain residual moisture do not take up the succeeding applications of dye at an uncontrolled rate.

From the foregoing description it will be readily seen that there has been produced a photographic

dye solution and process which substantially fulfills the objects of the invention as set forth herein.

While this specification sets forth the present and preferred details of the photographic dye solution and process, still in practice such deviations from such detail may be resorted to as do not form a departure from the spirit of the invention, as defined by the appended claims.

The dye identified herein as F. D. & C. Green No. 3 (Fast Green) (NAD), the last initials meaning National Aniline Division, is described on page 5 of the book entitled "Coal-Tar Regulations" of the Food & Drug Administration, said book having been issued September, 1940. The dye herein identified as F. D. & C. Blue No. 1 (NAD) is described in the British Colour Index on page 171 and the dye is identified by the dye number 671.

Having thus described the invention, the following is claimed as new and useful, and upon which Letters Patent are desired:

1. A stable dilute photographic dye solution for transferring a dye at a substantially uniform controlled rate into a photographic gelatin film, said solution having a pH close to the isoelectric point of gelatin and consisting essentially of a dilute aqueous solution of a dye, an aliphatic dihydroxy alcohol, acetic acid in amount capable of imparting to said dilute solution a pH of the order set forth, a wetting agent, and a hardening agent for the gelatin selected from the group consisting of acetaldehyde, paraldehyde, and aldol.
2. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid in amount sufficient to give the solution the pH stated, a wetting agent, and a hardening agent for the gelatin selected from the group consisting of acetaldehyde, paraldehyde and aldol.
3. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid imparting to said dilute solution a pH of the order set forth, a wetting agent, and a hardening agent for the gelatin selected from the group consisting of acetaldehyde, paraldehyde and aldol.
4. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, a wetting agent, and acetic acid imparting to said dilute solution a pH of the order set forth.
5. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid, acetaldehyde and sodium di-octyl sulfosuccinate acting as a wetting agent.
6. A stable dilute photographic dye solution for transferring a dye at a substantially uniform controlled rate into a photographic gelatin film, said solution having a pH close to the isoelectric

point of gelatin and consisting essentially of a dilute aqueous solution of a dye, diethylene glycol, a wetting agent, acetic acid imparting to said dilute solution a pH of the order set forth, the water content of the solution being less than the diethylene glycol content.

7. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid, acetaldehyde, a wetting agent to reduce the surface tension of the solution, the acetic acid being present in an amount to give 15 a solution having a pH near 4.43.

8. A stable dilute photographic dye solution for transferring a dye at a substantially uniform controlled rate into a photographic gelatin film, said solution having a pH close to the isoelectric 20 point of gelatin and consisting essentially of a dilute aqueous solution of a dye, diethylene glycol, a wetting agent to reduce the surface tension of the solution, acetic acid imparting to said solution a pH of the order set forth, and acetaldehyde, said solution having a slow hardening action on the gelatin.

9. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid imparting to said dilute solution a pH of the order set forth, a wetting agent to reduce the surface tension of the solution, and a polymer of the aldol condensation acting as a hardening agent for the gelatin.

10. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid imparting to said dilute solution a pH of the order set forth, a wetting agent to reduce the surface tension of the solution, and paraldehyde acting as a hardening agent for the gelatin.

11. A stable dilute photographic dye solution for transferring a dye at a substantially uniform controlled rate into a photographic gelatin film, said solution having a pH close to the isoelectric point of gelatin and consisting essentially of a dilute aqueous solution of a dye, diethylene glycol, acetic acid imparting to said dilute solution a pH of the order set forth, a wetting agent to reduce the surface tension of the solution, and aldol acting as a hardening agent for the gelatin.

12. A stable dilute photographic dye solution 60

for transferring a dye at a substantially uniform controlled rate into a photographic gelatin film, said solution consisting essentially of diethylene glycol, dilute acetic acid, and acetaldehyde, an aqueous solution containing a plurality of water soluble dyes of different colors, and a wetting agent, said solution having the three first named constituents thereof in substantially the following proportions:

|                                        | Volumes                                                                                                                                                                                                                                                                                         |
|----------------------------------------|-------------------------------------------------------------------------------------------------------------------------------------------------------------------------------------------------------------------------------------------------------------------------------------------------|
| Diethylene glycol                      | 2000                                                                                                                                                                                                                                                                                            |
| Dilute acetic acid (s. g. about 1.040) | 33.5                                                                                                                                                                                                                                                                                            |
| Acetaldehyde                           | 16                                                                                                                                                                                                                                                                                              |
| 30                                     | the volume of water in the solution being less than said volume of said glycol, and the amount of said wetting agent being sufficient to substantially reduce the surface tension of said solution, and the amount of the acetic acid being enough to give the dye solution a pH of about 4.43. |
| 35                                     | 13. A solution as covered in claim 12, in which the wetting agent is sodium di-octyl sulfosuccinate.                                                                                                                                                                                            |
| 40                                     | 14. A photographic dye solution which is an admixture of the following in the proportions stated:                                                                                                                                                                                               |
| 45                                     | 260 volumes of a solution of—<br>Dilute C. P. acetic acid, sp. gr. 1.040 33.5 cc.<br>Acetaldehyde 16 cc.<br>Diethylene glycol 2000 cc.                                                                                                                                                          |
| 50                                     | 60 volumes of a solution of—<br>Brilliant Scarlet 3R (C. I. 185)<br>(NAD) 100 grams.<br>Distilled water About 1000 cc.                                                                                                                                                                          |
| 55                                     | 35. 17 volumes of a solution of—<br>F. D. & C. Green No. 3 (Fast Green)<br>(NAD) 15 grams.<br>Distilled water About 1000 cc.                                                                                                                                                                    |
| 60                                     | 12 volumes of a solution of—<br>F. D. & C. Blue No. 1 (NAD) 15 grams.<br>Distilled water About 1000 cc.                                                                                                                                                                                         |
| 65                                     | 100 volumes of a solution of—<br>Aerosol OT 2 grams.<br>Distilled water About 1000 cc.                                                                                                                                                                                                          |
| 70                                     | such solution being stable, and being capable of transferring a dye at a substantially uniform controlled rate into a photographic gelatin film.                                                                                                                                                |

CLARENCE E. PAYNE.

References Cited in the file of this patent

UNITED STATES PATENTS

| Number       | Name       | Date          |
|--------------|------------|---------------|
| 1,582,136    | Gustin     | Apr. 27, 1926 |
| 55 1,652,949 | MacGivra   | Dec. 13, 1927 |
| 2,074,858    | Raffo      | Mar. 23, 1937 |
| 2,272,117    | Hasslacher | Feb. 3, 1942  |
| 2,433,811    | Haff       | Dec. 30, 1947 |
| 2,447,462    | Harsh      | Aug. 17, 1948 |